

# UNITED STATES PATENT OFFICE.

JOHN M. BURBY, OF ASTORIA, NEW YORK, ASSIGNOR TO THE PEMBEE COMPANY, OF NEW YORK, N. Y., A CORPORATION OF NEW YORK.

## PROCESS FOR THE RECOVERY OF PULP FROM WASTE PAPERS.

1,112,887.

Specification of Letters Patent.

Patented Oct. 6, 1914.

No Drawing.

Application filed June 15, 1911. Serial No. 633,417.

*To all whom it may concern:*

Be it known that I, JOHN M. BURBY, a citizen of the United States, and a resident of Astoria, Long Island, county of Queens, 5 and State of New York, have invented a certain new and useful Process for the Recovery of Pulp from Waste Papers, the following being a full specification thereof.

In the processes for the recovery of pulp 10 from printed waste papers, described in the literature and Letters Patent relating to the art, solvents are employed to dissolve or saponify the oily constituents of the printers' ink, and in some of them directions are given 15 to boil such waste papers in the stated solvents, or to subject them to the action of such solvents heated by steam under pressure, to reduce or destroy the adhesity of the ink, sizing, etc., to facilitate the separating of the 20 pulp fibers therefrom. The grades of paper, known collectively as print or "news print papers" and some grades of "book papers" are made partly—some of them largely—of wood fibers, produced by grinding 25 of raw wood. This material, known as the "mechanical wood pulp," differs from the "chemical" or "sulfite" pulp in that the fibers of this "mechanical" pulp, not having been subjected to the chemical process— 30 digesting—retain the nature of raw wood. When waste papers, made partly of this "mechanical" wood pulp, are subjected to the action of such, or as strong solvents as 35 are to be used in the processes heretofore known, or of such solvents heated, or under steam pressure, the raw wood fibers are discolored. This discoloration is very similar to that produced by exposing such papers to strong sunlight and cannot be obliterated, 40 because the fibers of mechanical wood pulp are detrimentally affected by bleaching, and liable to be rendered thereby wholly unfit to be used again, except probably as a filler. The more concentrated, or the hotter the 45 solvent is employed, the more intensive is its discoloring effect, and the larger the proportion of the mechanical wood pulp is contained in the waste papers, the more pro-

nounced is the discoloring effect upon all the pulp recovered. The fibers of the so-called 50 "chemical" pulp are not so discolored by these solvents, or by subjecting them to the action of such solvents in highly heated state, but as it is not practically feasible, to separate the fibers of this "chemical" pulp 55 from those of the "mechanical" pulp, the processes, heretofore known, cannot be employed for the recovery of pulp from waste papers containing a percentage of the mechanical wood pulp, because the pulp thus 60 recovered is reduced in quality to such an extent that it is no longer suitable for the manufacture of the same grade of paper for which it was originally used.

The object of this invention is to devise a 65 process to recover also the fibers of this so-called mechanical wood pulp, without their being discolored or their suitability for use in the manufacture of the same grade of paper otherwise impaired.

Alkalies are most suitable for use as solvents in processes for the recovery of pulp from printed waste papers, but if used in solutions containing more than the equivalent of two parts of caustic soda to one thousand 75 parts of water, or if weaker solutions are employed at a temperature of about 150° F., or more, they produce the explained discoloring effect upon the mechanical wood pulp which may be contained in such waste papers. I found, by an extended course of experiments, that a solution of one, or even less than one, part of caustic soda, measured by weight, in one thousand parts of water, if employed in proportionate quantities, is, in 80 most instances, sufficient to so diminish the adhesity of the oily medium of printers' ink, and of the sizing, that the pulp fibers can be readily separated therefrom, and that a solution containing less than two parts of 85 caustic soda, or its equivalent of other alkali, does not discolor the fibers of this mechanical pulp, unless heated to more than 150° F. Heating increases the intensity of 90 the action of such a weak solution and causes it to produce, to a degree, the stated 95

discoloring effect upon the fibers of the mechanical wood pulp.

In place of caustic soda, caustic potash may be used, and it should be noted, that 5 one and four-tenths parts of caustic potash are in these respects equivalent to one part of caustic soda; otherwise all said herein, as to the use and effect of caustic soda, applies equally to caustic potash. Other alkaline 10 solutions or compounds, as for instance, carbonates of soda and of potash, or ammonia, are effective in dissolving or saponifying the oily ingredients of printers' ink and of the 15 sizing, but they also have a similar discoloring effect upon the fibers of the mechanical wood pulp, if used in solutions containing more than the equivalent of two parts of caustic soda to one thousand parts 20 of water, or if a weaker solution of any of these alkalis is used hotter than 150° F. Also ammonia is not as effective in discoloring the fibers of mechanical wood pulp when used diluted proportionately to the 25 stated standard of two parts of caustic soda to one thousand parts of water. It is, however, not as certain in its effect upon the oily adhesive ingredients of printers' ink as the equivalent solutions of caustic potash or soda, or of their carbonates, and if 30 used in a stronger solution, is apt to produce a yet darker brown discoloration of the fibers of the mechanical wood pulp.

The process of recovering pulp from 35 printed waste papers, is best carried on, according to my invention, as follows: The waste papers are pulped in a beating engine and then conveyed to chests, provided with mechanical agitators. There a quantity 40 of the caustic soda solution is added thereto, so proportioned that, taking in consideration the quantity of water contained in the beaten stock, and which averages about twenty-nine thousand pounds to each 45 ton of such waste papers, there should be not more than two pounds of caustic soda, or its equivalent of some of the other alkalis, to one thousand pounds of water. It is necessary to explain, that in the course 50 of the process, a part of the alkali, contained in the solution, is consumed in saponifying the oily and adhesive ingredients of the ink and sizing. Taking, as a standard, a solution, containing one part of caustic soda 55 (or its equivalent of other alkali), to one thousand parts of water, this consumption of the alkali amounts to from thirty-three to forty-one per cent., if a quantity (weight) of the solution, equal to fifteen times the 60 weight of the paper stock treated, is used. The percentage of the consumption will be greater, if the solution is used in a smaller proportion, quantitatively, to the dry weight of the paper stock treated. Consequently,

a somewhat stronger or more concentrated 65 solution may be employed at the start of the process, provided that it be used in a sufficient quantity—not less than fifteen times the dry weight of the paper stock—as the strength of the solution is quite rapidly 70 diminished by the consumption of the alkali contained therein. When determining the initial strength of the solution, also the proportionate quantity of water, contained in the pulped material, when it is 75 run out from the beating engine, on the average of about fourteen and a half times its weight, must be taken in consideration as diminishing the strength of the solution added thereto. The pulped material is thoroughly 80 mixed and agitated in the solution and then the liquid is drained off, the pulped material conveyed upon movable screens and there washed with fresh clean water, whereby the carbon or other pigments, and other impurities, are removed, all traces of the alkali eliminated therefrom and the clean pulp fibers recovered. To avoid the difficulty, if there be any, in determining the proportionate quantity of 85 alkali to be used to produce a solution of only the requisite strength, the alkali may be dissolved in the water delivered into the beating engine and the waste papers subjected to the beating process; if this course 90 is followed, the pulped material need not be treated again in the chests, but should be soaked in fresh water and drained, before being conveyed upon the screens. The 95 pulp recovered from waste papers thus treated, may be conveyed to the paper making machine, or stored for future use; the fibers of the mechanical pulp contained therein are then and remain in such physical condition and color that the pulp can 100 be used again as it was recovered, without any further treatment, in the manufacture 105 of new paper of such a grade.

I claim as my invention:

1. The process of recovering the pulp 110 from printed waste papers made in part of mechanical wood pulp, the process consisting of the following steps: (1) pulping waste papers; (2) steeping the pulped material in a solution, made of not more than 115 two parts by weight of caustic soda, or its equivalent of other alkali, to one thousand parts of water at a temperature of not more than about 150° F. and agitating it therein; (3) washing the pulped material in 120 fresh water; and (4) separating the pulp fibers from all impurities, and collecting the cleaned pulp, substantially as herein set forth.

2. The process of recovering the pulp 125 from printed waste papers made in part of mechanical wood pulp, the process consisting of the following steps: (1) pulp-

ing the waste news print papers in a solution, made of not more than two parts by weight of caustic soda, or its equivalent of other alkali, to one thousand parts of water  
5 at a temperature of not more than about 150° F.; (2) soaking and washing the pulped material in fresh water; and (3)

separating the pulp from all impurities and collecting it; substantially as herein set forth.

JOHN M. BURBY.

Witnesses:

R. A. PIPER,  
VERONICA BRAUN.

---